

May 21, 1929.

F. A. J. FITZ GERALD

1,714,081

ELECTRIC FURNACE

Original Filed May 26, 1925 2 Sheets-Sheet 1



Fig. 1  
Inventor  
Francis A. J. Fitz Gerald  
By his Attorneys  
Edwards, Liger & Bower

May 21, 1929.

F. A. J. FITZ GERALD

1,714,081

ELECTRIC FURNACE

Original Filed May 26, 1925 2 Sheets-Sheet 2



Inventor

Francis A. J. Fitzgerald

By his Attorneys

Edwards, Lager & Bauer

Patented May 21, 1929.

1,714,081

# UNITED STATES PATENT OFFICE.

FRANCIS A. J. FITZ GERALD, OF NIAGARA FALLS, NEW YORK, ASSIGNOR TO HARPER ELECTRIC FURNACE CORPORATION, A CORPORATION OF NEW YORK.

## ELECTRIC FURNACE.

Original application filed May 26, 1925, Serial No. 32,879. Divided and this application filed May 13, 1927. Serial No. 191,046.

This invention relates to electric furnaces of the resistance type which may be used for heat treating substances and bodies of different kinds and forms in a variety of ways, such as curing, baking and glazing ceramic bodies; annealing, tempering, welding and fusing metal; and cremating, firing and burning materials and bodies.

Among the objects of my invention is to provide an improved electric furnace which shall be simple and economical in construction, durable in use, and which may be easily and efficiently operated.

In the preferred embodiment of my invention, I provide an electrically heated furnace wherein the resistors are contained within a closed heat chamber that may be kept filled with a gas, vapor or fume of such kind or quality as will render the resistors immune to, or protected from, deterioration such as may be caused by oxygen of the air or gases arising from the material being treated. The material or articles to be treated are contained in a chamber adjacent to the heat chamber but separated therefrom by a septum formed of material which is highly receptive, conductive and emissive of heat but is substantially non-reactive in the presence of atmospheric oxygen at high temperatures. The material forming the septum or division between the heat chamber and the chamber containing the material treated forms one of the important features of my invention. I preferably form the septum of silicon carbide such as carborundum, and particularly a form of silicon carbide which I will describe in detail hereafter. In the preferred form of my invention, I also line the walls of the heat chamber with this material so as to provide a path along which radiant heat received by the walls of the heat chamber may be conducted to the chamber containing the material treated.

Numerous objects and advantages of my invention will appear from the following description, taken in connection with the accompanying drawing, wherein

Fig. 1 is a view, partly in section on the line A of Fig. 2, partly in elevation and partly broken away, of a furnace disclosing one embodiment of my invention.

Fig. 2 is a section, partly broken away, taken on the line B of Fig. 1.

Fig. 3 is a transverse section on a some-

what enlarged scale taken on the line C of Fig. 1 and showing certain further details of construction.

Fig. 4 is a diagrammatic view of a preferred arrangement and disposal of the furnace resistor element or elements.

Referring to drawing, the heat-producing element 5 is preferably the so-called graphitized carbon zigzag resistor formed by cutting a series of blind-staggered slots 6 extending transversely of the block or slab. Graphitized carbon is a readily obtainable commercial commodity in regular sections up to 4 x 10 in. of from 4 to 6 ft. in length. For certain purposes it is preferable to machine or saw the sides at an angle as shown at 7 in Fig. 3 so as to give a greater radiating surface to the lower face 8 of the resistor 5. The resistor 5 is supported by means of carbonaceous terminals, 9, 10 as shown in Figs. 1, 2 and 3 projecting through the wall of the furnace. The connection between the terminals and resistor may be formed by a slip joint. If desired to secure adequate electrical connection with the terminals, such joint may be formed to provide a wedge fit, or such connections completed by packing with powdered graphite or carbonaceous material, not shown. In this manner, the resistor is supported between the terminal connections. When a resistor is desired of greater length than can readily be produced as a monolith, it is quite feasible to join two or more of such resistors together, end to end, as by capping their contiguous ends within the furnace; or, if desired, central terminal or terminals may be extended through the furnace walls and coupled together as shown in Fig. 4 outside of the furnace wall which is indicated by a dotted line 16 in Fig. 4. When arranged in this manner the two resistors may be operated in series from a source of current 12, or if it is desired to operate one of the resistors at a higher temperature than the other the connector block 13 between the adjacent terminals 9 and 10 of the two resistors may be removed and the resistors supplied from separate sources, as indicated at 14 and 15 in Fig. 4. With such an arrangement, if either resistor becomes inoperative, the other resistor can be run under a current 100

overload, thereby avoiding the loss of the charge.

The resistor chamber D is bounded by

relatively massive roof-slabs, or tiles, 17, side-slabs 18, 19 and floor plates 20, all being supported by another series of silicon carbide uprights 21 and foot-blocks 22, leaving 5 an interposed gap E connecting with an enlarged runway F, to receive a car, or series of cars, as 23, 24 and 25, mounted on wheels 26 and whose upper plates, or platforms, as 28 Figure 3, are also formed 10 of silicon carbide. The said floor plates 20, constitute a heat-transferring septum from the resistor chamber D, to the underlying conduit chamber H. Paralleling the outer surfaces of the chamber walls are wall gaps 15 filled with silicon carbide sand, 29. The outer roof may be suitably formed to receive pulverized, non-heat-conductive refractory material and the entire furnace may then be further enveloped with material most effective to 20 resist the outward flow of low-temperature heat, as indicated by the broken contour line 30.

It will now doubtless be apparent that the 25 path of least resistance for the flow of heat units from the lower surface of the resistor will be, as see arrows a, to and thence, by conduction, through the septum, from whence they proceed, by radiation, as see arrows b to the car-platforms and whatever may be 30 mounted thereon. Concurrently, however, and particularly from its sides, resistor heat will be imparted, as see arrows c, to the resistor chamber side walls, it being thence most freely conducted downwardly into the 35 supporting side walls, and foot blocks, escaping by radiation, as see arrows d, to the charge and the car platform. Naturally, a portion of the transferred energy is lost through the car-clearance spaces of the gap E; but the 40 actual sum of this, relative to the whole, is comparatively nominal and usually negligible.

As the mass of downwardly heat-conducting silicon carbide in the walls of the resistor chamber may be many times greater 45 than that of the resistor, and as these silicon carbide walls conduct the heat from the resistor with a comparatively small drop in temperature, and as this greater mass of silicon carbide serves as a heat reservoir, therefore fluctuations of temperature directly in and at the resistor itself are diminished. The transfer of heat units is rapid and efficient 50 notwithstanding the interposed septum, in that the septum is a good conductor of heat and sufficient difference in temperature between the resistor and the charge is permissible to obtain such transfer.

As a lining for the heat chamber and the chamber containing the material to be treated, I employ silicon carbide, preferably a form of silicon carbide which I prepare in the following manner. The silicon carbide carborundum in the form of grains or powder, as supplied commercially, is mixed with a

temporary binder such as flour paste or the like, and is then molded into the desired forms. The articles thus formed are then heated in an electric furnace to the temperature at which silicon carbide is formed, with 70 the result that recrystallization occurs and a dense, monolithic mass is obtained. The blocks, slabs or tiles so formed are then placed in the furnace structure in position to form the linings of the chambers and the septum 75 between the chambers and the furnace may then be heated in the usual manner so as to cause further recrystallization of the silicon carbide, thus causing adjacent blocks to coalesce, and the septum and chambers are 80 automatically formed devoid of joints. I have indicated the union of the joints by coalescence by wavy lines 31 and 32 in Fig. 3.

At the high temperature at which the furnace operates, oxygen must be excluded from 85 the chamber containing the resistor, or such chamber must contain a gaseous medium which will itself react with and wholly convert any oxygen which might otherwise reach the resistor and its juncture with the terminals. The inert gas may be introduced into the resistor chamber by means of a refractory tube 33, Fig. 3, and held under a head or pressure above that of atmosphere. In certain cases it is feasible to employ an enveloping 90 atmosphere of volatilized zinc, that is, zinc gas or zinc fume. The supply of this material can readily be maintained by an occasional introduction into the chamber D of molten zinc. In addition to its functioning as an 95 inert gas, zinc gas functions as an absorbing agent by being converted by any oxygen present to zinc oxide, which eventually fills all 100 crevices and prevents escape of the metal. Due to this self-sealing property, a nominal 105 renewal only of the zinc is required to maintain a sufficient quantity in the heat chamber, such renewal being merely such as to supply that lost by ventage-escape to avoid an 110 excessive development of pressure within the chamber. A further advantage of the use of the zinc gas is that it forms an effective heat-conductive agent.

Lower tubes 34, Figures 1 and 3, leading 115 to the conduit chamber, may serve a dual purpose; to permit the escape, or the withdrawal by suction, of air, gases and/or vapors; also to introduce gases and/or vapors, as for the purpose of producing reducing 120 atmospheres.

A plurality of cars, as 23, 24, 25 of Figure 1, each abutting upon another, may be continuously impelled through the furnace conduit at such a rate of motion that, to illustrate, when car 23 will have reached the position occupied by car 25, which is the hot zone of the conduit, the charge conveyed by that car will then be adequately heat-treated. If desired, as in the fusion of non-ferrous 125 metals, annealing iron, or heating steel for 130

hardening and tempering, the terminal ends of the conduit chamber may be enclosed and battened tightly, as at Z, Figure 1. Again, as in the case of ceramics, a dual furnace can 5 readily be constructed, each unit standing side by side, whereby the charge cars can readily be switched at the terminals, circulating through the chamber conduits with but a nominal heat loss from the cars themselves.

I find that the life of resistor or resistors, when operated according to the conditions above set forth, is practically interminable. Nevertheless, should a fracture occur, as from 15 accident or a very slow but progressive oxidation sufficient to eventually cause it to "sag" and pull apart, it will be perceived, by reference to Figures 1 and 3, that the upper or roof portion of the furnace can 20 readily be broken away, permitting a substitution of resistors even when the internal chamber-temperature is quite high.

Temperatures in this furnace can be readily controlled, for indefinite time periods, within 25 plus and minus tolerances of, say, 5° to 10° C.; but this condition is largely dependent upon pyrometry.

In certain cases, various modifications of the structure and method of operation above 30 described may be made. Thus, in certain cases a carbon or graphitized carbon resistor, even when of the zigzag form, will function satisfactorily if the space within its containing chamber is filled with silicon carbide, or with granular carbon or pulverized graphite. Again, the slab formed of angular 35 cross section of zigzag resistor need not necessarily be adhered to in that it may be cylindrical in transverse section, being encased 40 in a silicon carbide tube or otherwise formed.

It has been found that the graphite resistor can be greatly improved in its physical properties by undergoing heat treating process. This can be carried out by passing current of electricity through the resistor while 45 it is protected from oxidation so as to heat it to a temperature at least as high or considerably higher than that at which it will be used in actual practice. When this is done 50 it is found that the resistor is much tougher and more resilient than it was originally and consequently far less likely to be broken by

sudden changes in temperature or by external mechanical forces which would tend to break it.

This is a division of my co-pending application, Serial No. 32,879, filed May 26, 1925, for electric furnace.

I claim—

1. An electric furnace for heat treating substances having a resistor chamber containing an inert atmosphere, a heat treating chamber containing a gas having a pyrochemical and physical action on the substances heat treated and a septum between 65 said chambers that will not deteriorate when heated to a high temperature and subjected to a reducing atmosphere within the resistor chamber and a gas having a pyrochemical and physical action on the substances being 70 heat treated within the heat treating chamber.

2. An electric furnace for heat treating substances having a resistor chamber formed with a recrystallized silicon carbide lining 75 for said chamber containing a metallic gas, a heat treating chamber having means for introducing therein a gas having a pyrochemical and physical action on the substances heat treated and a recrystallized silicon carbide 80 septum between said chambers.

3. An electric furnace for heat treating substances having a resistor chamber containing an inert gas under pressure above that of atmosphere, a heat treating chamber, 85 means connected to said heat treating chamber for withdrawal or introduction of gases therein and a septum between said chambers preventing intermixture of the gases contained within said chambers but permitting 90 heat transfusion from the resistor chamber to the heat treating chamber.

4. An electric furnace for heat treating substances, a resistor chamber, a zigzag carbon resistor enclosed within said chamber, 95 means connected to said chamber for introducing into said chamber containing an inert zinc gas under pressure above that of atmosphere as an absorbing agent, a portion of which is adapted to be converted by any oxygen present within said chamber to zinc oxide 100 to form a seal for preventing escape of said gas.

FRANCIS A. J. FITZ GERALD.

**CERTIFICATE OF CORRECTION.**

Patent No. 1,714,081.

Granted May 21, 1929, to

**FRANCIS A. J. FITZ GERALD.**

It is hereby certified that error appears in the printed specification of the above numbered patent requiring correction as follows: Page 1, lines 59 and 60, for the misspelled word "furname" read "furnace"; line 67, for "commecial" read "commercial"; and lines 97 and 98, for "rasistors" read "resistors"; page 2, lines 63 and 64, strike out the word "carborundum"; page 3, line 97, claim 4, strike out the word "containing"; and that the said Letters Patent should be read with these corrections therein that the same may conform to the record of the case in the Patent Office.

Signed and sealed this 30th day of July, A. D. 1929.

(Seal)

**M. J. Moore,  
Acting Commissioner of Patents.**